

Oct. 21, 1924.

G. S. BROOKS

1,512,873

MANUFACTURE OF ZINC OXIDE

Filed Feb. 27, 1922

Fig. 2.



INVENTOR  
George S. Brooks  
By Lynnfield, Conant, Miles  
Attorneys

Patented Oct. 21, 1924.

1,512,873

# UNITED STATES PATENT OFFICE.

GEORGE S. BROOKS, OF GARY, INDIANA.

## MANUFACTURE OF ZINC OXIDE.

Application filed February 27, 1922. Serial No. 539,460.

*To all whom it may concern:*

Be it known that I, GEORGE S. BROOKS, a citizen of the United States, residing at Gary, in the county of Lake and State of Indiana, have invented a new and useful Improvement in the Manufacture of Zinc Oxide, of which the following is a specification.

The present invention relates to the manufacture of zinc oxide by the retort volatilizing, or French process and will be fully understood from the following description, illustrated by the accompanying drawing, in which a form of apparatus suitable for carrying out the invention is illustrated, in part diagrammatically.

In the manufacture of zinc oxide in accordance with the present invention, the usual form of retorts may be used, the mouths of which open into flues or passages in which a current of air is present, and wherein oxidation of the vapors of the zinc takes place. During the volatilization of the zinc, the volume of the zinc in the retort is completely or partially replenished by feeding fresh zinc into the retort, either from time to time or continuously at a rate not greater than the rate of volatilization of the zinc. In accordance with the present invention, it has been found desirable to employ for replenishment a spelter or metal containing not more than 0.07% of lead, the metal employed being preferably of the character of that obtained by electrodeposition from solutions of zinc salts derived directly from suitable zinc ores. The use of spelter of this character materially increases the length of runs and improves the character of the zinc oxide formed, permitting of full control of the latter.

The zinc metal to be retorted is preferably pre-formed in sheets or plates, say, of  $\frac{1}{16}$  to  $\frac{1}{4}$  inch thickness, in any suitable manner, for example, by electro-deposition from solutions derived from the lixiviation of suitable zinc ores. The zinc thus deposited is low in impurities, containing less than 0.07% lead.

The initially formed zinc plate is mechanically reduced to strip or sticks of a suitable size for introduction into the volatilizing retort, this being accomplished by means of any suitable device such as a mechanical shears.

55 The metal, in strip or stick form, is fed in at the mouth of the retort, from which

the zinc vapors are evolved and where the oxidation into oxide of zinc is effected. The in-fed metal is retained at or near the mouth of the retort in the heating zone created by the oxidation of the vaporized zinc, or by its superheat in case no oxidation is taking place, as for example, in the refining of zinc metal by retort volatilization. The sticks or strips of zinc may suitably be inserted into the retort from time to time, as the amount of zinc volatilized therefrom equals or exceeds the zinc of the strip or stick. In such case the strip may suitably be held in the heated zone outside the mouth of the retort prior to its introduction until it is brought to as high a temperature as possible, preferably just below its melting point. When so heated, it is inserted through the mouth of the retort and added to the molten metal for the replenishment of the latter. Cooling of the retort and the resulting injury to its material is thereby minimized and the regularity of the operation of the retort is disturbed as little as possible.

It is preferred, however, that the strips or sticks of zinc be fed continuously into the retort, passing through the heated zone due to zinc oxide formation or super-heat of the zinc vapors prior to entering the mouth of the retort. In such case the rate of feed of the strips or sticks is so controlled that, in passing through the heated zone, the metal of the strips or sticks is brought to the highest possible temperature below the melting point of the zinc, the zinc metal becoming plastic and, as it enters the retort, bending downward of its own weight to meet the level of the molten zinc in the retort. By such continuous feed of the zinc meal, a continuous and regular operation of the retort may be maintained, particularly when using a metal of the character above described containing not more than 0.07% of lead.

In the drawings, apparatus is shown which may suitably be used for the continuous feeding, for example, of strips into the volatilizing furnace.

Fig. 1 is a sectional view through the retort, showing the feeding mechanism in plan;

Fig. 2 is a sectional view on the line 2—2 of Fig. 1, and

Fig. 3 is a detail sectional view through the feeding nozzle on a slightly enlarged scale.

In the drawings, the numeral 5 indicates

a retort provided at its mouth with a dam 7 and mounted in a suitable furnace setting 8. The mouth of the retort opens into a suitable flue or conduit 9 through which air 6 may be drawn in the manufacture of the oxide, combining with the zinc vapors issuing from the mouth of the retort and forming zinc oxide, which passes upwardly through the conduit or flue into suitable settling chambers or bag houses (not shown). Opposite the mouth of the retort 6 a water-cooled nozzle 10 protrudes into the flue 9, the nozzle opening being of a width and thickness suitable for passage through it, 15 for example, of a mechanically cut strip of spelter from an electrolytically deposited plate of, say, about  $\frac{1}{8}$  of an inch thickness. The nozzle forms the end of suitable feeding mechanism mounted upon a wheeled carriage 11 suspended from a trolley, which may suitably be an I-beam 12. The feeding mechanism illustrated consists of a frame 13 upon which are mounted feeding rollers 14—14 and idle rolls 15 for feeding 20 and guiding the strips to and through the nozzle. Any suitable driving mechanism may be employed for the feed rolls 14. The end of the nozzle 10 is fed at a point outside the mouth of the retort 6 at which the full 25 heating effect of the zinc oxide flame issuing from the mouth of the retort is felt. The zinc strips are slowly fed through the zinc oxide flame, the rate being so controlled that they approach their melting point, becoming very plastic and bending downward 30 to meet the surface of the molten zinc in the retort, as shown at 16.

I claim:

1. In the process of producing zinc oxide 40 by volatilizing zinc metal in a retort and oxidizing the volatilized zinc upon leaving the retort, the improvement which consists in feeding solid zinc metal into the retort during the volatilization through the heating zone formed by the oxidizing flame, the in-fed zinc being subjected to the heating ac-

tion of the flame for a sufficient period to effect a substantial heating thereof.

2. In the process of producing zinc oxide by volatilizing zinc metal in a retort and 50 oxidizing the volatilized zinc upon leaving the retort, the improvement which consists in feeding solid zinc metal into the retort during the volatilization through the heating zone formed by the oxidizing flame, the in-fed zinc being subjected to the heating 55 action of the flame for a sufficient period of time to bring it substantially to the melting point of the zinc.

3. In the process of producing zinc oxide 60 by volatilizing zinc metal in a retort and oxidizing the volatilized zinc upon leaving the retort, the improvement which consists in continuously feeding solid zinc metal into the retort during the volatilization through 65 the heating zone formed by the oxidizing flame, the rate of feed of the in-fed zinc being such that the zinc metal is brought substantially to its melting point upon entering the retort. 70

4. In the retort volatilization of zinc, maintaining a substantial body of molten zinc in a volatilizing retort and continuously feeding solid zinc into the retort at a rate to substantially replace the zinc vola- 75 tilized therefrom.

5. In the retort volatilization of zinc, maintaining a substantial body of molten zinc in a volatilizing retort and continuously feeding solid zinc into the retort 80 through the vapors issuing therefrom at a rate to substantially replace the zinc volatilized therefrom, the in-fed zinc being thereby preheated.

6. In the retort volatilization of zinc, 85 maintaining a substantial body of molten zinc in a volatilizing retort, feeding solid zinc into the retort through the vapors issuing therefrom, and retaining the in-fed zinc in said vapors during the feeding to effect 90 a substantial preheating thereof.

GEORGE S. BROOKS.